

# UNITED STATES PATENT OFFICE.

HANS GROSSMANN, OF OBER-URDORF, NEAR ZURICH, SWITZERLAND.

## PLASTIC INSULATING COMPOSITION.

1,183,640.

Specification of Letters Patent.

Patented May 16, 1916.

No Drawing.

Application filed August 5, 1914. Serial No. 855,302.

To all whom it may concern:

Be it known that I, HANS GROSSMANN, analytical chemist, a citizen of Switzerland, residing at Ober-Urdorf, near Zurich, Switzerland, have invented new and useful Improvements in Plastic Insulating Compositions, of which the following is a specification.

The hitherto known filling and insulating materials, that is, insulating materials capable of being cast for electrotechnical purposes, have up till now only been put on the market in the form of solid blocks which, before they can be used, have to be ground down with considerable expenditure of power and time for the purpose of melting.

The present invention relates to a filling and insulating material which obviates the above-named drawbacks as this material is put on the market in powder form, that is, in the most favorable condition for melting.

The new molding and insulating material consists at least of a resinous substance of low melting point and a substance which increases the insulating properties of the material and which does not fuse at the melting point of the resinous substance, the two said substances being intimately mixed with one another.

The easily fusible resinous material may be, for example, resin, pitch, asphalt or the like, while the other substance, which increases the insulating properties, may be, for example, glass, porcelain, marble, talc, sand, heavy spar or the like. The latter substance also fulfills incidentally the further purpose of maintaining the material in powder form, since the resinous material when pulverized very easily fuses or cakes together when kept for a long time. For the preparation of the filling and insulating material, both substances are intimately mixed with one another in a finely powdered form. For example, 50% of powdered colophonium and 50% of pulverized glass may be employed for the mixture. The relative quantities of the two substances can, however, be altered within wide limits, according to the nature of the substances used and the particular purpose or use desired.

By alteration of the relative quantities it is possible to also regulate the melting point of the mixture within wide limits.

The material prepared from the two substances mentioned exhibits a certain brittleness after fusing and subsequent solidifying, which brittleness may be disadvantageous in certain cases. In order to lessen or entirely obviate this brittleness, a quantity of easily fusible ductile material also in powder form may be added with advantage. This material may be, for example, paraffin wax, carnauba wax, montan wax or the like, and the quantity used may also be varied within fairly wide limits.

Assuming the above named substances to be used, the following proportions for the mixture may be used:

|      |                           |    |
|------|---------------------------|----|
| I.   | 45% powdered colophonium. | 70 |
|      | 45% powdered glass.       |    |
|      | 10% powdered paraffin.    |    |
| II.  | 30% powdered colophonium. |    |
|      | 60% powdered glass.       |    |
|      | 10% powdered paraffin.    |    |
| III. | 60% powdered colophonium. | 75 |
|      | 25% powdered glass.       |    |
|      | 15% powdered paraffin.    |    |

The filling and insulating material described permits of a much simpler and more convenient handling in use than the molding and insulating materials hitherto used. The new filling and insulating material also offers the further advantage that it can be produced at less cost.

I claim:

1. The herein described filling and insulating material for electrotechnical purposes consisting of powdered colophonium, powdered glass, and powdered wax; all substances being intimately mixed together, substantially as set forth.

2. The herein described filling and insulating material for electrotechnical purposes consisting of about 30 to 60% powdered colophonium, 25 to 60% powdered glass, and 10 to 15% paraffin wax; all substances being intimately mixed together, substantially as described.

3. The herein described filling and insu-

100

80

85

90

95

100

lating material for electrical purposes, consisting of forty-five per cent. of powdered colophonium, forty-five per cent. of powdered glass, and ten per cent. of paraffin  
5 wax, said material being mixed together in powdered form, and adapted to be heated to form a plastic mass.

In testimony whereof I have signed my name to this specification in the presence of two subscribing witnesses.

HANS GROSSMANN.

Witnesses:

CONRAD BOLTSHAMER,  
CAN CUESRIN.

Copies of this patent may be obtained for five cents each, by addressing the "Commissioner of Patents,  
Washington, D. C."